# EUROPEAN PATENT APPLICATION

(11) **EP 1 004 942 A1**
(43) Date of publication of application: **31.05.2000**
(21) Application number: 99203837.2
(22) Date of filing: 17.11.1999
(51) Int. Cl.: G03G 9/113

(54) **A hybrid carrier coating containing a silane network and a polymeric compound not containing silicon atoms.**

(30) Priority: 26.11.1998 EP 98204006
(71) Applicant: AGFA-GEVAERT N.V., 2640 Mortsel (BE)
(72) Inventor: Tavernier, Serge, Agfa-Gevaert N.V., 2640 Mortsel (BE); Heitzmann, Daniel, Agfa-Gevaert N.V., 2640 Mortsel (BE)

(57) **Abstract**

Carrier particles having a coating comprising a polycondensation network containing a chemical compound selected from the group consisting of a monomeric polyfunctional organosilane, an hydrolysis product of a monomeric polyfunctional organosilane, a reaction product of a monomeric polyfunctional organosilane with an organosilane containing an hetero-atom and a reaction product of a monomeric polyfunctional organosilane with an alkoxide,
characterised in that
the coating further comprises between 5 % and 50%, by weight, both limits included, of a polymeric compound not containing silicon atoms.

## Description

### FIELD OF THE INVENTION

This invention relates to coated particles. It relates especially to coated carrier particles to be used as carrier particles in multi-component developers for electrostatic imaging with magnetic brush development as well in cascade development.

### BACKGROUND OF THE INVENTION

In electrostatographic imaging carrier particles, mostly magnetic carrier particles, are mixed with toner particles (and with other ingredients) to form a developer. When the developer is to be used in magnetic brush development, the carrier particles are magnetic, when the developer is used in cascade development, the carrier particles can be coated glass beads. In any case the rubbing of the carrier particles and the toner particles induce a tribo-electric charge in the toner particles and the nature of the coating on the carrier particles determines, together with the toner ingredients, not only the polarity of the charge on the toner articles and the amount of the charge but also the stability of the charge over time, the charge distribution over the population of toner particles, etc. Thus the coating of the carrier particles is very crucial to the resulting properties of the developer and thus to the image quality that can be reached with that developer. Also the speed of charging of the toner particles is to a large extent determined by the coating of the carrier particles. Carrier particles having an high speed of charging towards the toner particles are beneficial especially when images with high image fill (i.e. a high amount of area in an page is really occupied by toning particles) are present. Then large amounts of toner are consumed and the toner, especially in long run printing, resides only a limited time in the developer. In such a situation the toner has only a limited number of activation cycles. Hence the charging properties of the developer, in terms of its kinetics, i.e. the speed of the rise of the charge amount, as well as in terms of its plateau value are important.

In **JP-A-10 153 886** it is disclosed to apply on carrier particles for use in electrostatograpohic developers a coating of a polyester with relatively high acid value and tri-alkyloxysilane compounds that contain groups that can react with the free acid groups of the polyester.

In **WO-A 98/53372** a new type of coating has been described, consisting of chemical compounds selected from the group consisting of a monomeric polyfunctional organosilane, an hydrolysis product of a monomeric polyfunctional organosilane, a reaction product of a monomeric polyfunctional organosilane with an organosilane containing an hetero-atom and a reaction product of a monomeric, polyfunctional organosilane with an alkoxide. Such a coating offers interesting properties as described in said application. Moreover in **EP-A 898 206** it has been disclosed that such a coating could be applied to carrier particles in a quite simple method that requires only mechanical stirring and uses a quite low amount of solvents.

The coating disclosed in **WO-A 98/53372** combined with the method described in **EP-A 898 206** has a very long lifetime and can easily be manufactured in an inexpensive method. However is showed that the coating shows some limitations in terms of activation behaviour, i.e. the charging of the toner particles in rubbing contact with the carrier coating shows relatively low speed and thus when images with high page fill have to be printed, some problems with charging can occur.

There is thus a further need for improvement in activation property for such coatings. Moreover it has been found that this tendency is quite general. Silicon-atom containing coatings seem to have a lower activation property, and so it is described in literature, to add charging agents to such coatings. At the same time it is observed that the incorporation of these charging agents gives some instabilities the manufacturing method described previously. In particular coagulation and/or agglomeration happens to some extent, thus giving rise to composition differences in the coating and hence differences in properties of the coated particles.

There is thus still a need to improve the performance of coated particles in general and carrier particles.

### OBJECTS AND SUMMARY OF THE INVENTION

It is an object of the invention to provide a coating composition whereby the coating can be designed in a flexible way to incorporate new properties and performances in this coating especially with respect to the speed of charging.

It is a further object of the invention to provide a coating composition whereby said coating can be applied in a easy, inexpensive and controllable way, resulting in a thin homogeneous layer without interruptions on the surface of the particles.

It is a further object of the invention to provide a coating composition whereby said coating can be applied in such a way that the composition of said coating on different particles of said coated particles population is similar to a high extent, inducing similar properties all over the coated particles and that during coating no or very few agglomerates are formed.

Further objects and advantages of the invention will become clear from the detailed description hereinafter.

The objects of the invention are realised by providing carrier particles having a coating comprising a polycondensation network having moieties derived from chemical compounds selected from the group consisting of a monomeric polyfunctional organosilane, an organosilane containing an hetero-atom and an alkoxide,
characterised in that
said coating further comprises an amount A of a polymeric compound not containing silicon atoms so that 5% ≤ A ≤ 50 % by weight, with respect to the weight of the dried coating.

### DETAILED DESCRIPTION OF THE INVENTION

The quality of a coating for carrier particles according to the chemistry disclosed in WO-A 98/53372, that is included herein by reference, could surprisingly be enhanced with respect to the activation, i.e. the speed of charge accumulation on toner particles by rubbing contact between the carrier and the toner particles, when appreciable amounts of a non silicon containing polymeric substance were included in the coating. It was found that between 5 and 50 % by weight, both limits included, of such non silicon containing polymeric compounds could be incorporated in the coating. Preferably an amount between 10 and 30 % by right, both limits included, is incorporated. Very surprisingly it showed possible to incorporate such amounts of non silicon containing polymeric compounds in the coating using the method that was disclosed in EP-A 898 206 without problems of agglomeration and in a very reproducible way, although when said method was used for coating the particles with the same non silicon containing compound alone severe agglomeration occurred. It seems, without being bound to any theory that the non silicon containing polymeric compound is kind of trapped in the polycondensation network forming a complex or an interpenetrating network.

Thus carrier particles according to this invention comprise a coating comprising a polycondensation network having moieties derived from chemical compounds selected from the group consisting of a monomeric polyfunctional organosilane, an organosilane containing an hetero-atom and an alkoxide,
characterised in that
said coating further comprises an amount A of a polymeric compound not containing silicon atoms so that 5% ≤ A ≤ 50 % by weight, with respect to the weight of the dried coating.

In a preferred embodiment, said polycondensation network is derived from 20 to 80 % by weight of polyfunctional organosilane, 20 to 80 % by weight of alkoxide, 0 to 10 % by weight of organosilane (I) which contains a hetero atom. In a more preferred embodiment, said polycondensation network contains 19.9 to 80 % by weight of polyfunctional organosilane, 19.9 to 80 % by weight of alkoxide (II), 0.1 to 10 % by weight of organosilane (I) which contains a hetero atom.

The polycondensation network can in addition to the chemicals above contain finely divided metal oxides or metal oxide-hydroxides of the elements Si, Sn, In, Tl, Zr, B or Al, e.g. silica sols, which contain organic solvents in particular. The preferred primary particle size thereof falls within the range from 1 to 50 nm; they are hereinafter termed "nanoparticles".

When nano-particles are incorporated ion the polycondensation network, it is preferred that said polycondensation network contains moieties derived from 0.1 to 100 % by weight of polyfunctional organosilane, 0 to 20 % by weight of organosilane (I) which contains a hetero atom, 0 to 99.9 % by weight of alkoxide (II) and 0 to 70 % by weight of nano-particles a. In a more preferred embodiment, said polycondensation network contains 20 to 80 % by weight of polyfunctional organosilane, 20 to 80 % by weight of alkoxide (II), 0 to 10 % by weight of organosilane (I) which contains a hetero atom, and 0 to 50 % by weight of nano-particles.

### The non silicon containing polymeric compound

The non silicon containing polymeric compound has preferably an average molecular weight by number larger than 1000, more preferably larger than 2000. It can be addition home-polymers ,e.g., polystyrene, polymethylacrylate, polymethylmethacrylate, polymethylacrylicacid, polymethylmethacrylacid, etc.. It can be copolymers as, e.g., styreneacrylic resins. It can also be vinylpolymers as polyvinylbutyral, polyvinyl acetate, polyvinylalcohol, etc.. The vinyl polymers are preferred as non silicon containing polymer for use in the present invention. Also polycondensation polymers, e.g., polyesters, polyamides, polyimides etc. can be used as well as polymers comprising fluor containing moieties.

### The organosilane containing an hetero-atom

The organosilane containing an hetero-atom for use in a carrier coating according to this invention consist of at least one silicon atom carrying an hydrolysable group and/or a group that can be cross-linked by polycondensation and at least on organic rest group, bound to the silicon atom by a carbon atom, wherein the rest group contains an hetero atom and can be an alkyl, cycloalkyl or aryl group. silicon atom carrying an hydrolysable group and/or a group that can be cross-linked by polycondensation can be -SiOR, wherein R can be an alkyl, cycloalkyl or aryl group and is preferably an alkyl group or -SiOH. It is preferred that R is an alkyl group. The hetero atoms can be N, P, S, F, Cl, Br, O, B and Al, but are more preferably N or F.

Very preferred nitrogen containing organosilane for use in a coating according to this invention have the formula (I) :

(R₂)₂-N[(CH₂)ₘNR₂]ₙ(CH₂)ₘSi(OR₃)₃₋ₒ(R₄)ₒ (I)

wherein 1 ≤ m ≤ 10, preferably m = 2 or 3, 0 ≤ n ≤ 2 preferably n = 2, 0 ≤ o ≤ 2, preferably o = 0, R₂ is hydrogen, alkyl or aryl, preferably hydrogen, R₃, R₄ that are equal or different are alkyl or aryl groups, preferably CH₃ or C₂H₅.

Typical useful nitrogen containing alkoxysilane are :
H₂N-(CH₂)₃Si(OCH₃)₃
H₂N-(CH₂)₃Si(OC₂H₅)₃
H₂N-(CH₂)₂-HN-(CH₂)₃Si(OCH₃)₃
H₂N-(CH₂)₂-HN-(CH₂)₃Si(OCH₃)₂CH₃
C6H5-HN-(CH₂)₃Si(OCH₃)₃
C6H5-HN-(CH₂)₃Si(OC₂H₅)₃
H₂N-(CH₂)₂- HN-(CH₂)₂-HN-(CH₂)₃Si(OCH₃)₃
H₂N-(CH₂)₂- HN-(CH₂)₂-HN-(CH₂)₃Si(O C₂H₅)₃

Typical useful nitrogen containing alkoxysilane are :
F₃C-(CH₂)₂SiR'₃₋ₓ(OR)ₓ
F₃C-(CF₂)₇-(CH₂)₂SiR'₃₋ₓ(OR)ₓ
(F₃C)₂CF-O-(CH₂)₃SiR'₃₋ₓ(OR)ₓ
(3-F₃C-C₆H₄)-SiR'₃₋ₓ(OR)ₓ
(3-F₃C-C₆H₄)₂-Si(OR)₂
wherein 1 ≤ x ≤ 3, R, R' equal or different are alkyl, cycloalkyl or aryl, preferably R and R' are either methyl or ethyl.

### The alkoxide

The alkoxide for use in a coating according to this invention corresponds preferably to formula (II) :

M₁(OR₁)_{y} (II)

Wherein
M₁ = Si, Sn, Ti, Zr, B , P or Al
R₁ = alkyl or aryl, preferably a C1 to C4 alkyl, more preferably CH₃ or C₂H₅.
y = 4 when M₁ = Si, Sn, Ti, Zr, y = 3 when M₁ = B , P or Al.

Preferred alkoxides are Si(OC₂H₅)₄, B(OC₂H₅)₃, Al(O-i-C₃H₇)₃ and Zr(O-i-C₃H₇)₄. It is highly preferred to use Si(OC₂H₅)₄ as alkoxide in a polycondensation network on the carrier particles of this invention.

### The polyfunctional organosilane

Polyfunctional organosilanes for use in the present invention comprise at least 2, preferably 3 Si-atoms coupled to 1 to 3 hydrolysable groups and/or a group that can be cross-linked by polycondensation. The latter groups are preferably alkoxy-, acyloxy or hydroxygroups. The Si-atoms are preferably coupled by a Si-C bond to an organic group, e.g., to a linear or branched C1 to C10 alkylgroup, to a C5 to C10 cycloalkylgroup, to an aromatic group or combinations of these.
Polyfunctional organosilanes useful to prepare a coating according to this invention correspond to formula (III), (IV) and (V)

(R₅)₄₋ᵢSi[(CH₂)ₚSi(OR₆)ₐ(R₇)₃₋ₐ]ᵢ (III)

wherein
i is an integer with value between 2 and 4, preferably i = 2
p is an integer with value between 1 and 4, preferably 2 ≤ p ≤ 4
a is an integer with value between 1 and 3
R₅ is an alkyl or aryl group
R₆ hydrogen, alkyl or aryl when a = 1
R₆ alkyl or aryl when a = 2 or a = 3
R₇ alkyl or aryl, preferably methyl.
wherein
m is an integer with value between 3 and 6, preferably m = 3
q is an integer with value between 2 and 10, preferably q =2
b is an integer with value between 1 and 3
R₈ is a C1-C6 alkyl or C6-C14 aryl group, preferably CH₃, C₂H₅
R₉ hydrogen, alkyl or aryl, preferably H, CR₃, C₂H₅, C₃H₇ when c = 1
R₉ alkyl or aryl, CH₃, C₂H₅, C₃H₇ when c = 2 or c = 3
R₁₀ alkyl or aryl, preferably methyl.

(R₁₄)₄₋ₖSi[OSi(R₁₁)₂Si(OR₁₂)_{c}(R₁₃)_{3-c}]ₖ (V)

wherein
k is an integer with value between 2 and 4, preferably i = 4
r is an integer with value between 1 and 10, preferably 2 ≤ p ≤ 4
c is an integer with value between 1 and 3
R₁₄ is an alkyl or aryl group
R₁₂ hydrogen, alkyl or aryl, preferably H, CH₃, C₂H₅, C₃H₇ when c = 1
R₁₂ alkyl or aryl, CH₃, C₂H₅, C₃H₇ when c = 2 or c = 3
R₁₁ alkyl or aryl, preferably methyl.

Typical examples of polyfunctional organo silane useful in this invention are :
Si[(CH₂)₂Si(OH)(CH₃)₂]₄
H₃C Si[(CH₂)₂Si(OH)(CH₃)₂]₃
H₆C₅Si[(CH₂)₂Si(OH)(CH₃)₂]₃
Si[(CH₂)₃Si(OH)(CH₃)₂]₄
cyclo-{OSiCH₃[(CH₂)₂Si(OH)(CH₃)₂]}₄
cyclo-{OSiCH₃[(CH₂)₂Si(O CH₃)(CH₃)₂]}₄
cyclo-{OSiCH₃[(CH₂)₂Si(O CH₃)₂CH₃]}₄
cyclo-{OSiCH₃[(CH₂)₂Si(O C₂H₅)₂CH₃]}₄
cyclo-{OSiCH₃[(CH₂)₂Si(O C₂H₅)₃]}₄

### The coating solution

It is preferred to prepare a coating solution with the chemical compounds described above by adding an amount between 0.1 to 50 % by weight of a polyfunctional organosilane and 0 to 50 % of an alkoxide optionally together with a catalyser, which can be an organic acid e.g. formic acid, acetic acid, paratoluenesulphonic acid, etc. in a solvent ( preferably a lower C1 to C4 alcohol, most preferred isopropanol). After a pre-reaction 0 to 20 % by weight of a organosilane containing an hetero-atom is added and the solution is further diluted with solvent. Then with 2.5 to 25 % by weight of a polymeric compound non containing silicon atoms is added. In a further preferred embodiment said coating solution comprises 5 to 15 % of a polymeric compound non containing silicon atoms.

In a further preferred embodiment said coating solution comprises between 30 and 50 % by weight of a polyfunctional organosilane reacted with between 30 and 50 % by weight of alkylorthosilicate (preferably tetraethylorthosilicate = TEOS = (Si(OC₂H₅)₄), between 0 and 5 % of an organo silane comprising an hetero atom and between 5 and 15 % by weight of a polymeric compound non containing silicon atoms.

The relative amounts of the constituents of the coating are adapted so has to have a total of 100 %.

When this solution is coated on the particles and dried the polyfunctional organosilane, the alkoxide and the organosilane containing an hetero-atom have reacted together and have lost water and alcohol so that in the dried coating only 50 % by weight of sum of the amounts (weight) of the polyfunctional organosilane, the alkoxide and the organosilane added to the coating solution is contained in the coating. The non silicon atom containing polymer does not loose weight during the coating and thus when 2.5 % by weight of the non silicon atom containing polymer is added to the coating solution, 5 % by weight is present in the dried coating.

The present invention thus encompasses a method for coating carrier particles with a polycondensation network incorporating a polymer not containing Si-atoms, comprising the steps of :
mixing an amount between 0.1 to 50 % by weight, with respect to the total amount of chemicals used for forming said polycondensation network, of a polyfunctional organosilane and 0 to 50 %, with respect to the total amount of chemicals used for forming said polycondensation network, of an alkoxide, optionally together with a catalyser in a lower C1 to C4 alcohol forming a coating solution,
adding 0 to 20 % by weight, with respect to the total amount of chemicals used for forming said polycondensation network, of a organosilane containing an hetero-atom to said solution,
diluting said solution further with said lower C1 to C4 alcohol
mixing between 2.5 to 25 % by weight, with respect to the total amount of chemicals used in said coating solution, of a polymeric compound non containing silicon atoms in said solution,
applying said solution to said carrier particles forming a layer of said solution on said particles and
drying said particles.

Preferably in said step of mixing a polyfunctional organosilane and an alkoxide between 30 and 50 % by weight, with respect to the total amount of chemicals used for forming said polycondensation network, of said polyfunctional organosilane are mixed with between 30 and 50 % by weight, with respect to the total amount of chemicals used for forming said polycondensation network, of an alkylorthosilicate and in said step of adding a organosilane containing an hetero-atom 0 and 5 % by weight, with respect to the total amount of chemicals used for forming said polycondensation network, of an organo silane comprising an hetero atom are added.

In a further preferred embodiment, in said step of mixing a polyfunctional organosilane and an alkylorthosilicate, said alkylorthosilicate is tetraethylorthosimlicate (TEOS) and in said step of mixing a polymeric compound non containing silicon atoms in said solution between 5 and 15 % by weight, with respect to the total amount of chemical in said coating solution of said polymeric compound non containing silicon atoms are used.

The coating solution according to this invention and described immediately above can preferably be applied to the carrier particles by the method disclosed in EP-A 898 206 and its equivalent US-A-5 888 692, that is incorporated herein by reference.

The present invention encompasses thus also a method for coating carrier particles, having a volume average diameter between 20 and 200 µm, for use in electrostatic developers, comprising the steps of :
- bringing said carrier particles to be coated in a vessel equipped with means for agitating said carrier particles , so that said carrier particles occupy less than 85 % by volume of said vessel, and the agitation of the carrier particles is described by a Froude number between 0.2 and 20,
- adding a solution containing between 6 and 60 % by weight with respect to the total volume of said solution of chemical compounds for coating said carrier particles in a solvent with a boiling point of A °C to said vessel at such a rate that, at any time, said solvent is present in an mount lover than 1.25 10⁻⁴ ml per cm² of surface of said carrier particles to be coated ,
- keeping said carrier particles in said vessel at a temperature of at most (A + 10) °C, and
- continuously evacuating said solvent,
   characterised in that
   said solution of chemical compounds contains of a polymeric compound not containing silicon atoms and a chemical compound selected from the group consisting of a monomeric polyfunctional organosilane, an hydrolysis product of a monomeric polyfunctional organosilane, a reaction product of a monomeric polyfunctional organosilane with an organosilane containing an hetero-atom and a reaction product of a monomeric polyfunctional organosilane with an alkoxide
   said polymeric compound not containing silicon atoms is present in said solution for between 5 and 50 % by weight with respect to the total weight of chemical compounds in said solution.

Preferably said Froude number is between 0.5 and 8 both limits included.
Said solution with chemical compounds for coating the carrier particles contains preferably between 15 and 40 % by weight with respect to the total volume of said solution of chemical compounds for coating said particles.
Said solution is preferably added to said vessel at a rate that, at any time, said solvent is present in an amount lover than 0.6 10⁻⁴ ml per cm² of surface of said particles to be coated.
In a preferred embodiment of this invention, said vessel with a mechanical mixer wherein the carrier particles are coated is a ploughshare mixer.
Carrier particles coated with a coating composition according to this invention, can be used in any multi-component developer comprising magnetic carrier particles and toner particles, it can be used in electrophotography, direct electrostatic printing, ionography etc.

### EXAMPLES

### 1. Toner particles

The toner used for the experiment had the following composition : 97 parts of a co-polyester resin of fumaric acid and propoxylated bisphenol A, having an acid value of 18 and volume resistivity of 5.1 x 10¹⁶ Ω.cm was melt-blended for 30 minutes at 110° C in a laboratory kneader with 3 parts of Cu-phthalocyanine pigment (Colour Index PB 15:3). A resistivity decreasing substance - having the following structural formula : (CH₃)₃N⁺C₁₆H₃₃Br⁻ - was added in a quantity of 0.5 % with respect to the binder.

After cooling, the solidified mass was pulverised and milled using an ALPINE Fliessbettgegenstrahlmühle type 100AFG (trade name) and further classified using an ALPINE multiplex zig-zag classifier type 100MZR (trade name). The resulting particle size distribution of the separated toner, measured by Coulter Counter model Multisizer (trade name), was found to be 6.3 µm average by number and 8.2 µm average by volume. In order to improve the flowability of the toner mass, the toner particles were mixed with 0.5 % of hydrophobic colloidal silica particles (BET-value 130 m²/g).
An electrostatographic developer was prepared by mixing said mixture of toner particles and colloidal silica in a 4 % ratio (wt/wt) with carrier particles coated according to the examples.

### 2. Coating of the carrier particles

7.5 kg of ferrite beads, having an average volume diameter dᵥ of 50 µm. Were placed in a vessel equipped with a stirrer. A coating solution is prepared and is added over 25 minutes at 80 °C. The mixtures are post-cured during 120 minutes at 140 °C. Then the amount of agglomerates is determined by sieving over a 125µm sieve and expressed as % wt/wt. The charging characteristics are measured upon admixture of 5% of toner. The Q/M-value is determined at different activation times, by a blow-off method. The difference of the Q/M-values is taken as an indication of the activation property of the coated carrier particles.

### COMPARATIVE EXAMPLE 1

A coating solution is prepared containing 39.7 g of cyclo-{OSiCH₃[(CH₂)₂Si(O C₂H₅)₂CH₃]}₄ and 37 g of TEOS (Si(OC₂H₅)₄), in 15 g of isopropanol and 6.6 g of a 0.1 N solution of paratoluenesulphonic acid as a catalyst. After one hour at room temperature, 0.39 g of H₂N-(CH₂)₂-HN-(CH₂)₂-HN-(CH2)₃Si(OCH₃)₃ is added together with 150 g of isopropanol. This results, after reaction and coating in 38.5 grams of a polycondensation network. This solution was added to the ferrite beads in the general coating procedure described above so as to have a dry coating of 0.5 % by weight with respect to the weight of the ferrite beads.
In this comparative example, wherein NO non silicone containing polymeric compound is added, the number of agglomerates was 2 % and the Q/m (charge over mass ratio) as a function of rubbing time is given in the table below :

| Rubbing time | Q/m |
|---|---|
| 2 min | 13.3 |
| 10 min | 14.1 |
| 30 min | 16.0 |
| 60 min | 18.4 |

It is seen that the Q/m ratio is not a constant and increases over the time, thus showing a lower speed of charging.

### COMPARATIVE EXAMPLE 2

In this example the ferrite beads were coated according the general procedure above with a solution containing ONLY non silicone containing polymeric compound. In his case BUTVAR B79 (trade name of polyvinyl butyral from Monsanto),weight average molecular weight Mw = 34000-38000 was used. The coating solution consisted of 15% BUTVAR in a mixture 1/3 MEK-2/3 isopropanol. Amount of coated material is 0.5% relatively to ferrite carrier core.
In this example 50 % of agglomerates were found and when the carrier beads were mixed with the toner particles no stable charge measurements could be done.

### INVENTION EXAMPLE 1

Comparative example 1 was repeated, except for the fact that 5 % by weight of BUTVAR B79 (trade name of polyvinyl butyral from Monsanto),weight average molecular weight Mw = 34000-38000 was added to the coating solution before coating, resulting in a coating containing 10 % by weight of BUTVAR and 90 % by weight of the polycondensation network.
In this invention example, wherein a non silicone containing polymeric compound is added, the number of agglomerates was 6 % and the Q/m (charge over mass ratio) as a function of rubbing time is given in the table below :

| Rubbing time | Q/m |
|---|---|
| 2 min | 18.0 |
| 10 min | 16.9 |
| 30 min | 17.9 |
| 60 min | 19.0 |

It is seen that the maximum Q/m ratio almost reached after 2 minutes and remain fairly constant. Thus these carrier particles show a high speed of charging.

### INVENTION EXAMPLE 2

Invention example 1 was repeated but a dispersion of carbon black (KETJEN BLACK EC) is added so that in the final coating contained 20 % by weight of Carbon Black, 20 % by weight of BUTVAR B79 and 60 % by weight of the polycondensation network.
In this invention example, wherein a non silicone containing polymeric compound and a charge regulating agent is added, the number of agglomerates was 3 % and the Q/m (charge over mass ratio) as a function of rubbing time is given in the table below :

| Rubbing time | Q/m |
|---|---|
| 2 min | 15.2 |
| 10 min | 15.0 |
| 30 min | 14.4 |
| 60 min | 15.7 |

It is seen that the maximum Q/m ratio almost reached after 2 minutes and remain fairly constant. Thus these carrier particles show a high speed of charging.

## Claims

1. Carrier particles having a coating comprising a polycondensation network having moieties derived from chemical compounds selected from the group consisting of a monomeric polyfunctional organosilane, an organosilane containing an hetero-atom and an alkoxide, characterised in that
said coating further comprises a relative amount, A, of a polymeric compound not containing silicon atoms so that 5 % ≤ A ≤ 50 % by weight, with respect to the weight of the dried coating.

2. Carrier particles according to claim 1, wherein 10 % ≤ A ≤ 30 % by weight.

3. Carrier particles according to claim 1 or 2 wherein said polymer compound not containing silicon atoms is a member selected from the group consisting of acrylic resins, vinyl resins, fluor containing addition polymers, polyesters, polyimides and polyamides.

4. Carrier particles according to claim 1 or 2 wherein said polymer compound not containing silicon atoms is a member selected from the group consisting of polyvinylbutyral, polyvinylacetate and polyvinylalcohol.

5. Carrier particles according to claims 1 to 4, wherein said polycondensation network contains moieties derived from 19.9 to 80 % by weight of said polyfunctional organosilane, 19.9 to 80 % by weight of said alkoxide , 0.1 to 10 % by weight of said organosilane which contains a hetero atom.

6. Carrier particles according to claim 5 wherein said alkoxide is an alkylorthosilicate.

7. Carrier particles according to claim 6 wherein said alkylorthosilicate is tetraethylorthosilicate, TEOS.

8. A method for coating carrier particles with a polycondensation network incorporating a polymer not containing Si-atoms, comprising the steps of :
mixing an amount between 0.1 to 50 % by weight, with respect to the total amount of chemicals used for forming said polycondensation network, of a polyfunctional organosilane and 0 to 50 %, with respect to the total amount of chemicals used for forming said polycondensation network, of an alkoxide, optionally together with a catalyser in a lower C1 to C4 alcohol forming a coating solution,
adding 0 to 20 % by weight, with respect to the total amount of chemicals used for forming said polycondensation network, of a organosilane containing an hetero-atom to said solution,
diluting said solution further with said lower C1 to C4 alcohol
mixing between 2.5 to 25 % by weight, with respect to the total amount of chemicals used in said coating solution, of a polymeric compound non containing silicon atoms in said solution,
applying said solution to said carrier particles forming a layer of said solution on said particles and
drying said particles.

9. A method for coating carrier particles, having a volume average diameter between 20 and 200 µm, for use in electrostatic developers, comprising the steps of :
- bringing said carrier particles to be coated in a vessel equipped with means for agitating said carrier particles , so that said carrier particles occupy less than 85 % by volume of said vessel, and the agitation of the carrier particles is described by a Froude number between 0.2 and 20,
- adding a solution containing between 6 and 60 % by weight with respect to the total volume of said solution of chemical compounds for coating said carrier particles in a solvent with a boiling point of A °C to said vessel at such a rate that, at any time, said solvent is present in an amount lower than 1.25 10⁻⁴ ml per cm² of surface of said carrier particles to be coated ,
- keeping said carrier particles in said vessel at a temperature of at most (A + 10) °C, and
- continuously evacuating said solvent,
characterised in that
said solution of chemical compounds contains of a polymeric compound not containing silicon atoms and a chemical compound selected from the group consisting of a monomeric polyfunctional organosilane, an hydrolysis product of a monomeric polyfunctional organosilane, a reaction product of a monomeric polyfunctional organosilane with an organosilane containing an hetero-atom and a reaction product of a monomeric polyfunctional organosilane with an alkoxide and
said polymeric compound not containing silicon atoms is present in said solution for between 2.5 and 25 % by weight with respect to the total weight of chemical compounds in said solution.

10. A method according to claim 9 wherein said solution comprises between 0.1 to 50 % by weight of a polyfunctional organosilane, between 0 to 50 % by weight of an alkoxide and between 0 to 20 % by weight of a organosilane containing an hetero-atom.

11. A method according to claim 9, wherein said coating solution comprises between 30 and 50 % by weight of a polyfunctional organosilane, between 30 and 50 % by weight of alkylorthosilicate, between 0 and 5 % of an organo silane comprising an hetero atom and between 5 and 15 % by weight of a polymeric compound not containing silicon atoms.

12. A method according to any of claim 9 to 11, wherein said solution contains further a catalyser selected from the group consisting of formic acid, acetic acid and paratoluenesulphonic acid.
